# EUROPEAN PATENT APPLICATION

(11) **EP 4 775 693 A1**
(43) Date of publication of application: **15.07.2026**
(21) Application number: 24862190.6
(22) Date of filing: 05.09.2024
(51) Int. Cl.: C14C 1/00

(54) **METHOD FOR PRODUCING LEATHER, AND LEATHER PRECURSOR**

(30) Priority: 07.09.2023 JP 2023145525
(71) Applicant: S.R. Leather Pte. Ltd., Singapore 179097 (SG)
(72) Inventor: SAKURAI, Kazushige, Aisai-shi, Aichi 496-8015 (JP); PURNOMO, Eddy, Mungkid Magerang, 56513 (ID)
(74) Representative: Scott, Stephen John
(86) International application number: PCT/IB2024/058620
(87) International publication number: WO 2025/052280

(57) **Abstract**

Provided are a method for producing leather and a leather precursor that have a low environmental impact. The method for producing leather includes a soaking process of immersing a raw hide in a treatment liquid containing a sugar and a yeast of the genus Saccharomyces, and a first fermentation process of immersing the raw hide in the treatment liquid and fermenting. The leather precursor includes a sugar, a yeast of the genus Saccharomyces, and a raw hide.

## Description

### TECHNICAL FIELD

The present disclosure relates to a method for producing leather and to a leather precursor.

### BACKGROUND

Leather is produced by cleaning raw hides, removing fat and hair, and then tanning treatment. The process of processing raw hides into leather may involve transportation from where the raw hides are collected to a processing plant. For transport to the processing plant, curing treatment such as salting with salt is applied in order to prevent change in quality or degradation, such as putrefaction, of the raw hides. Further, during the processing into leather, processing treatments are carried out such as soaking, which removes salt from the raw hides subjected to a curing treatment (leather precursor), and liming, which removes hair and unnecessary protein from the treated hides. These processing treatments generate wastewater containing large amounts of salt and lime, resulting in a large environmental burden.

In Patent Literature (PTL) 1, which concerns a method for preserving raw hides using salt, a problem is pointed out that a large amount of salt is required to preserve raw hides, and that waste liquid discharged from storage buildings and tanneries is heavily contaminated with soluble salt. Further, it is pointed out that salt in waste liquid is difficult to remove without incurring substantial costs, and that in some countries, used salt is classified as hazardous waste. Further, it is pointed out that salt-resistant bacteria can spoil treated hides, and that the amount of salt needed to preserve raw hides for short periods is almost the same as that needed for long-term preservation.

In PTL 2, a problem is pointed out in a method for producing leather, where hides are stirred with slaked lime and water to remove hair and loosen hide fibers, but this results in the generation of a large amount of sludge, the main component of which is slaked lime containing hair and the like that has separated from the hides, which must be disposed of as alkaline sludge. In relation to this problem, PTL 2 describes a method for producing leather that is capable of decreasing the amount of sludge containing slaked lime as a main component, and slaked lime used in the method. This method for producing leather includes a process of treating animal hides with slaked lime, and when producing leather from the treated hides, a specific surface area of the slaked lime is set within a defined range. In PTL 2, an example is described of a dehairing process in this method for producing leather, in which soaking and fleshing treatments are carried out on five pieces of salted pig hide, and after completely removing salt, meat fragments, and the like, the dehairing process is carried out. In this dehairing process, the fleshed hides (total weight 23.5 kg), water (200 % relative to the fleshed hides), and slaked lime (2 % relative to the fleshed hides, 0.47 kg) are placed in a stainless steel drum and stirred by rotation. While being stirred, sodium sulfide (2 %) and a nonionic surfactant (0.3 %) are added in that order, and the mixture is then stirred overnight. Further, in PTL 2, an example is described of a reliming process after the dehairing process. In this reliming process, grain-side hides (total weight 18.8 kg), water (200 % relative to the hides), and slaked lime (1 % relative to the hides, 0.188 kg) are placed in the same drum as used during dehairing and stirred, followed by the addition of a nonionic surfactant (0.3 %), and then the mixture is stirred for two days and nights.

In PTL 3, the following are described: an antioxidant fermentation microbial agent used to reduce odors and volatile organic compounds generated from leather products, leather containing the agent, and a method for producing same. This antioxidant fermentation microbial agent contains salt such as natural deep-sea salt. This method for producing leather uses hides that have been preserved with salt, and the salt needs to be removed during production of the leather. Further, this method for producing leather uses a saturated aqueous solution of lime for dehairing the hides.

In PTL 4, a method for preserving baked bakery products is described. The method includes, after a process of baking the dough, applying a solution containing a live fermentation starter and/or live yeast onto the surface of the baked bakery product. An example of a yeast for this method is a strain of Saccharomyces cerevisiae.

### CITATION LIST

### Patent Literature

PTL 1: JP S62-600 A
PTL 2: JP 2000-045000 A
PTL 3: WO 2007/12986 A1
PTL 4: JP 2023-504068 A

### SUMMARY

### (Technical Problem)

According to the conventional methods for producing leather described in PTL 1 to PTL 3, a large amount of salt (table salt, sodium chloride) is used to preserve the raw hides, and waste liquid containing a large amount of salt is generated during the production of leather, which places a heavy burden on the environment. Further, large amounts of lime are used in intermediate processes in processing raw hides into leather (such as dehairing and loosening skin fibers), resulting in waste liquid containing large amounts of lime, which places a heavy burden on the environment. Therefore, it is desirable to provide a method for producing leather and a leather precursor that place less of a burden on the environment.

The present disclosure is made in view of the above circumstances, and it would be helpful to provide a method for producing leather and a leather precursor that have a low environmental impact.

### (Solution to Problem)

The method for producing leather according to the present disclosure comprises:
a soaking process of immersing a raw hide in a treatment liquid containing a sugar and a yeast of the genus Saccharomyces; and
a first fermentation process of immersing the raw hide in the treatment liquid and fermenting.

The leather precursor according to the present disclosure comprises:
a sugar; a yeast of the genus Saccharomyces; and a raw hide.

### (Advantageous Effect)

According to the present disclosure, it is possible to provide a method for producing leather and a leather precursor that have a low environmental impact.

### DETAILED DESCRIPTION

The following describes a method for producing leather and a leather precursor according to an embodiment of the present disclosure. First, outlines of the method for producing leather and the leather precursor according to the present embodiment are described.

The method for producing leather according to the present embodiment includes a soaking process of immersing a raw hide in a treatment liquid containing a sugar and a yeast of the genus Saccharomyces, and a first fermentation process of immersing the raw hide in this treatment liquid and fermenting.

The leather precursor according to the present embodiment contains a sugar, a yeast of the genus Saccharomyces, and a raw hide.

According to the method for producing leather according to the present embodiment, it is possible to produce leather precursors and leather with a reduced environmental impact.

Specifically, the method for producing leather according to the present embodiment has the following effects. In the method for producing leather according to the present embodiment, there is no need to use salt to preserve the raw hide during production. In other words, the method for producing leather according to the present embodiment makes it possible to preserve a raw hide at the site of collection and during transportation from the site of collection to a processing plant without using salt. According to the present embodiment, preserving or preservation treatment of a raw hide means preventing a change in quality or degradation, such as putrefaction, of the raw hide. Therefore, in the method for producing leather according to the present embodiment, it is not necessary to use a raw hide that has been salted as a curing treatment, and it is also not necessary to remove salt from the raw hide. Therefore, the method for producing leather according to the present embodiment does not generate waste liquid containing a large amount of salt during the production of leather, and therefore has a low environmental impact.

The method for producing leather according to the present embodiment can also realize hide dehairing with reduced environmental impact (hereinafter referred to as the method for dehairing hide according to the present embodiment).

The method for dehairing hide according to the present embodiment includes a soaking process of immersing a raw hide in a treatment liquid containing a sugar and a yeast of the genus Saccharomyces, and a first fermentation process of immersing the raw hide in this treatment liquid and fermenting. The raw hide used must not have been salted.

Specifically, the method for dehairing hide according to the present embodiment has the following effects. In the method for dehairing hide according to the present embodiment, dehairing can be carried out without using a large amount of water or a large amount of lime (slaked lime, calcium hydroxide). Therefore, the method for dehairing hide according to the present embodiment does not discharge large amounts of lime sludge as in conventional techniques, and has a low environmental impact.

That is, the method for producing leather according to the present embodiment includes a process realizing the method for dehairing hide according to the present embodiment. In the following description, the method for dehairing hide according to the present embodiment is described as being included in the description of the method for producing leather according to the present embodiment.

The method for producing leather and the leather precursor according to the present embodiment are described in detail below.

In the method for producing leather according to the present embodiment, the concept of leather includes preserved raw hide (an example of a leather precursor), hide obtained by dehairing preserved raw hide (another example of a leather precursor), hide obtained by tanning preserved raw hide (another example of a leather precursor), leather, and leather products. The leather precursor according to the present embodiment is raw hide that has been at least subjected to a preservation treatment and processed (for example, dehaired or tanned). In other words, the leather precursor of the present embodiment is hide in the process of being processed into leather (which has been subjected to preservation treatment), and is an intermediate in the process of being processed into leather.

As an example, the method for producing leather according to the present embodiment may further include, in addition to the soaking process and the first fermentation process described above, a dewatering process in which a first-stage precursor obtained by fermenting raw hide in the fermentation process is dewatered, a sugar addition process in which sugar is attached to a surface of the first-stage precursor after the dewatering process, a second fermentation process in which the first-stage precursor after the sugar addition process is fermented, a dehairing process in which a second-stage precursor obtained by fermenting the first-stage precursor in the second fermentation process is dehaired, and a desulfurization process carried out after the dehairing process.

In each process described above, the first-stage precursor and the second-stage precursor before the dehairing process are included in the leather precursor according to the present embodiment.

According to the present embodiment, the raw hide may be a hide obtained from animals such as cows, buffalo, pigs, wild boars, goats, sheep, lizards, snakes, crocodiles, and fish. The raw hide may be obtained, for example, as a residual when the animal is slaughtered for meat processing. A certain amount of meat may remain on the raw hide. The raw hide may have animal hair remaining on a front surface (body surface side, animal hair side). As a raw hide collected from an animal, use of a raw hide that has been salted is not required. Preferably, the raw hide is not salted. After initial washing, the raw hide is subjected to a soaking process, which is described later.

During the initial washing, dirt adhering to the raw hide taken from the animal is removed, unnecessary parts such as legs and tail are cut off, and meat and fat are removed using a fleshing machine or the like. During the initial washing, disinfectant (but not salt) may be used to prevent early contamination or rapid putrefaction. After washing, the raw hide is not salted.

The soaking process is a process in which the raw hide is immersed in a treatment liquid. The treatment liquid contains a sugar and a yeast of the genus Saccharomyces. The dispersion medium or solvent of the treatment liquid may be water.

An example of the yeast of the genus Saccharomyces is Saccharomyces cerevisiae. Saccharomyces cerevisiae may be that included in so-called baker's yeast, glutinous rice yeast, or cassava yeast.

The yeast of the genus Saccharomyces used in the treatment liquid may be a mixture of yeasts from a plurality of origins. For example, 100 parts by weight of baker's yeast containing Saccharomyces cerevisiae may be mixed with 10 parts by weight to 50 parts by weight, preferably 30 parts by weight, of other yeast containing Saccharomyces cerevisiae, such as glutinous rice yeast or cassava yeast, and this mixture may be used as the mixture of yeasts of the genus Saccharomyces used in the treatment liquid.

The yeast serves as a fermenting microbe in the first fermentation process and the second fermentation process described below. Yeast metabolizes sugar, described later, to undergo alcoholic fermentation.

The sugar may be any sugar that can undergo alcoholic fermentation by the yeast. Examples of suitable sugars according to the present embodiment include glucose, fructose, and sucrose. The sugar does not need to be pure, and may be molasses, Java sugar fructose, palm sugar fructose, tapioca sugar, or granulated sugar containing any of these as a main component, provided the sugar contains at least one of glucose, fructose, or sucrose.

The treatment liquid may be prepared by mixing water containing sugar with a starter. The starter is a yeast that has been pre-fermented with a small amount of sugar and water.

The soaking of the raw hide in the treatment liquid, that is, the soaking process, may be carried out, for example, as follows.

First, the weight of the raw hide is measured after the initial washing. The weight of the raw hide includes the weight of volatile substances (such as water) that the raw hide may naturally contain. Next, pretreatment is carried out by immersion in a pretreatment liquid containing soap or antibacterial agent (a cleaning agent having antibacterial properties, excluding salt) and soda ash (sodium carbonate) for 5 minutes to 30 minutes, preferably 10 minutes to 15 minutes. The hydrogen ion concentration index (pH) of the pretreatment liquid is weakly alkaline, that is, pH 7 to pH 9, and preferably pH 8 to pH 9.

Separately from the pretreatment, a starter is prepared. The starter is prepared by fermenting a defined amount of yeast and a defined amount of sugar in warm water.

The starter can be prepared by placing 3 g to 15 g, preferably 5 g to 10 g, of yeast and 3 g to 15 g, preferably 5 g to 10 g, of sugar into a container containing 20 ml to 100 ml of warm water (35 °C to 65 °C), and allowing fermentation for at least 10 minutes, preferably 15 minutes to 20 minutes, with the container sealed. The starter is preferably prepared by fermenting the liquid in the container until the liquid becomes foamy.

The amount of warm water used to prepare the starter is preferably 30 ml to 70 ml, more preferably 40 ml to 60 ml. The temperature of the hot water used to prepare the starter is preferably 40 °C to 60 °C.

Then, water of a weight equivalent to that of the raw hide, specifically water of a weight of 50 % to 200 % of the weight of the raw hide (at room temperature, for example, 25 °C), is measured out, and sugar of a weight of 1.5 % to 30 % of the weight of the raw hide is added to the water and dissolved to form a sugar solution.

The amount of water used to prepare the sugar solution is preferably 50 % to 120 % of the weight of the raw hide, and more preferably 50 % to 100 %.

The temperature of the water when preparing the sugar solution is suitably 20 °C to 35 °C, and preferably 20 °C to 30 °C.

The sugar used in preparing the sugar solution may be, for example, the granulated sugar described above. The amount of sugar used in preparing the sugar solution is preferably 3 % to 30 % of the weight of the raw hide, and more preferably 5 % to 30 %.

After preparing the sugar solution, the entire amount of the starter is added to the sugar solution to prepare the treatment liquid. The treatment liquid is preferably stirred after the starter is added. The starter may be added to the sugar solution to which the pretreated raw hide has been added, or to the sugar solution to which the pretreated raw hide has not been added.

The treatment liquid prepared as described above may contain water that is 50 % to 200 % of the weight of the raw hide, and sugar that is 1.5 % to 30 % of the weight of the raw hide. When the treatment liquid has such a component ratio, the treatment liquid may be more effective in preventing a change in quality or degradation, such as putrefaction, of the raw hide. Further, by using a treatment liquid that has such a component ratio, it may be possible to shorten the time required to prevent a change in quality or degradation, such as putrefaction, of the raw hide, that is, a holding time (fermentation time) required in the first fermentation process.

The amount of water contained in the treatment liquid is preferably 50 % to 120 % of the weight of the raw hide, and more preferably 50 % to 110 %. The amount of water in the treatment liquid is sufficient as long as the raw hide remains immersed in the treatment liquid even after the treatment liquid has permeated the raw hide.

The amount of sugar contained in the treatment liquid is preferably 3 % to 30 % of the weight of the raw hide, and more preferably 5 % to 30 %. The amount of sugar contained in the treatment liquid may be increased when the amount of water contained in the treatment liquid is increased, and may be decreased when the amount of water contained in the treatment liquid is decreased. The ratio of water to sugar in the treatment liquid is preferably 4.2 % to 60 %, relative to the weight of water contained in the treatment liquid.

The starter is not essential for preparing the treatment liquid. For example, yeast may be directly added to a sugar solution, and the sugar solution containing the yeast may be pre-fermented to prepare the treatment liquid.

The pretreated raw hide is immersed (soaked) in the treatment liquid prepared as described above. According to the present embodiment, immersing the raw hide in the treatment liquid means that the treatment liquid is applied to at least the entire surface of the raw hide. The soaking of the raw hide in the treatment liquid may be carried out in a rotating drum. The drum may be, for example, a cylindrical drum having a horizontal rotation axis and a diameter of 2 m to 4 m. An example of the rotation speed of the drum is 5 revolutions per minute to 30 revolutions per minute, preferably 6 revolutions per minute to 10 revolutions per minute.

Soaking the raw hide in the treatment liquid in a rotating drum can sometimes result in better coverage of the treatment liquid over the entire surface of the raw hide. Further, the treatment liquid (starter and sugar solution) can be stirred sufficiently. These factors may allow the fermentation in the first fermentation process described below to proceed more efficiently throughout the raw hide.

The first fermentation process is the first process in which the raw hide immersed in the treatment liquid is fermented. In the first fermentation process, the raw hide is kept immersed in the treatment liquid. This allows the treatment liquid to penetrate into the raw hide, and yeast grows in the treatment liquid and in the raw hide (within the hide tissue), and fermentation proceeds. That is, the first fermentation process is a process in which the raw hide is kept immersed in the treatment liquid for fermentation.

In the first fermentation process, the concept of keeping the raw hide immersed in the treatment liquid includes both a case where the treatment liquid and the immersed raw hide are stationary and a case where the treatment liquid and the immersed raw hide are moving, for example, due to stirring. In the first fermentation process, fermentation proceeds as long as the raw hide is immersed in the treatment liquid.

In the first fermentation process, ethanol is produced in the treatment liquid and in the raw hide by the fermentation. That is, the first-stage precursor is raw hide containing sugar and yeast of the genus Saccharomyces. The first-stage precursor raw hide is preferably free of salt added for preservation purposes. The first-stage precursor may also contain ethanol, depending on the fermentation conditions. According to the present embodiment, salt contained in the raw hide as biological tissue from the time of collection is not included in the concept of salt added for preservation purposes.

In the first fermentation process, the raw hide is kept immersed in the treatment liquid for 2 hours to 72 hours, preferably 3 hours to 15 hours, more preferably 4 hours to 15 hours, and even more preferably 12 hours to 15 hours, and fermented.

According to the present embodiment, the raw hide that has undergone the first fermentation process is referred to as the first-stage precursor. That is, the first-stage precursor is raw hide that has been subjected to the first fermentation process. More specifically, raw hide that has undergone the first fermentation process (the first-stage precursor) is raw hide that has been immersed in the treatment liquid through the soaking process, and is raw hide from the point at which fermentation in the first fermentation process has begun. Unless the raw hide is handled in an atmosphere that inhibits the progress of fermentation (for example, when refrigerated to an extent that fermentation stops), the point at which the raw hide is immersed in the treatment liquid during the soaking process may be the start of the first fermentation process.

In this way, by subjecting the raw hide to the first fermentation process, an effect of preservation treatment is exerted, to prevent a change in quality or degradation, such as putrefaction, of the raw hide. The first fermentation process is a process for preventing a change in quality or degradation, such as putrefaction, of the raw hide (the first-stage precursor). Further, the first fermentation process is a process for exerting an effect of preventing a change in quality or degradation, such as putrefaction, of the first-stage precursor after the first fermentation process.

By setting the holding time (fermentation time) in the first fermentation process to two hours or longer, that is, by immersing the raw hide in the treatment liquid and allowing fermentation for two hours or longer, the treatment liquid (yeast) for which fermentation has proceeded sufficiently penetrates into the raw hide, and the effect of the preservation treatment of preventing a change in quality or degradation, such as putrefaction, of the raw hide (the first-stage precursor) is more effectively exerted. Further, conditions are created in the raw hide that facilitate fermentation, enhancing the effectiveness of the preservation treatment. Further, the effect of the preservation treatment of the first-stage precursor continues even after the first fermentation process is completed.

When the holding time (fermentation time) in the first fermentation process is four hours or longer, such as when the raw hide is immersed in the treatment liquid and left to ferment for 12 hours, fermentation progresses sufficiently in the raw hide.

The atmosphere in the room, warehouse, or the like where the first fermentation process is carried out may be such that the temperature is 15 °C to 40 °C, and the relative humidity is 30 % to 80 %. The atmosphere preferably has a temperature of 15 °C to 30 °C and a relative humidity of 30 % to 80 %, and more preferably a temperature of 20 °C to 30 °C and a relative humidity of 60 % or less. By carrying out the first fermentation process in such an atmosphere, fermentation is promoted in the treatment liquid and the raw hide, thereby further enhancing the effectiveness of the preservation treatment to prevent a change in quality or degradation, such as putrefaction, of the raw hide (the first-stage precursor).

In the first fermentation process, when the raw hide has animal hair, an effect of making the animal hair of the first-stage precursor more likely to detach is also achieved. That is, the method for dehairing hide according to the present embodiment may include the first fermentation process. In the first fermentation process, some animal hair detaches as the fermentation progresses. This facilitates the dehairing process (finishing dehairing process) described below.

The first-stage precursor is brought into a state in which putrefaction-promoting microorganisms (hereinafter referred to simply as "microorganisms") are unlikely to proliferate, due to ethanol produced by the yeast metabolizing sugar and due to the growth of the yeast or the yeast that has proliferated. That is, the first-stage precursor is one in which the progression of putrefaction is inhibited even without the use of salt. Hereinafter, inhibition of the progression of putrefaction may be referred to as being cured, or the like. Further, inhibiting the progression of putrefaction may be referred to as curing, or the like.

The first-stage precursor has progression of putrefaction inhibited as described above, and therefore can be preserved for some days to a week, for example, when raw hide is transported between plants. As described above, no salt is required in the production of the first-stage precursor. Therefore, wastewater containing a large amount of salt is not generated in the production of the first-stage precursor.

According to the present embodiment, the first-stage precursor may be further subjected to the second fermentation process. The second fermentation process is a process in which the first-stage precursor is further fermented.

To carry out the second fermentation process, it is preferable to provide additional sugar for the yeast to metabolize. According to the present embodiment, the first-stage precursor may be subjected to the second fermentation process after the sugar addition process of attaching sugar to the surface of the first-stage precursor.

According to the present embodiment, the dewatering process of dewatering the first-stage precursor may be carried out prior to the sugar addition process and the second fermentation process. According to the present embodiment, dewatering refers to removing a portion of a liquid component from the first-stage precursor. According to the present embodiment, the liquid component contained in the first-stage precursor is mainly the treatment liquid after fermentation has progressed (mainly water).

The dewatering of the first-stage precursor in the dewatering process may be carried out by squeezing the first-stage precursor. The dewatering of the first-stage precursor in the dewatering process may be carried out using, for example, a sammying machine, a press, or a centrifuge. By squeezing out a certain amount of liquid component (water) from the first-stage precursor in the dewatering process, it becomes easier for sugar to adhere to the surface of the first-stage precursor in the sugar addition process. Further, the dewatering process can suppress the growth of microorganisms. Further, by attaching sugar to the first-stage precursor after dewatering, free water in the first-stage precursor can be reduced, and the proliferation of various microorganisms can be inhibited. That is, the dewatering process allows for better curing.

The dewatering ratio (squeezing ratio) in the dewatering process is preferably 40 % to 60 %. The dewatering ratio (squeezing ratio) is the ratio (%) of the weight of removed water to the weight of the first-stage precursor immediately before dewatering, which is taken as 100 %. That is, in the dewatering process, it is preferable to remove a liquid component of 40 % to 60 % by weight of the first-stage precursor.

In the sugar addition process, the attachment of sugar to the surface of the first-stage precursor may be carried out by coating or applying sugar particles (powder or granules) onto the surface of the first-stage precursor. Alternatively, the attachment of sugar to the surface of the first-stage precursor may be carried out by applying a sugar paste in which sugar is dissolved at a high concentration onto the surface of the first-stage precursor. When sugar paste is used, the sugar concentration in the sugar paste is preferably 10 % by weight or more, more preferably 20 % by weight or more.

The sugar attached to the surface of the first-stage precursor in the sugar addition process is a sugar (second sugar) prepared separately from the sugar (first sugar) contained in the treatment liquid. In other words, the concept of sugar attached to the surface of the first-stage precursor in the sugar addition process does not include the sugar in the treatment liquid remaining on the surface of the first-stage precursor.

The sugars that can be used in the second fermentation process are the same as those listed as examples of sugars that can be used in the treatment liquid in the first fermentation process. The sugar contained in the treatment liquid and the sugar attached to the surface of the first-stage precursor do not need to have different components or be different types. The sugar contained in the treatment liquid and the sugar attached to the surface of the first-stage precursor may be the same component or type, or may be different components or types.

The attachment of sugar to the surface of the first-stage precursor may be carried out on at least one of the front surface (epidermis, animal hair surface) or the back surface (dermis) of the hide. The attachment of sugar to the surface of the first-stage precursor is preferably carried out on the back surface. The back surface of the first-stage precursor has larger irregularities than the front surface, making it suitable for attaching sugar.

In the sugar addition process, an antimicrobial agent may be added together with the sugar. When an antimicrobial agent is added, it is sufficient to add an amount of 0.3 % by weight to 1.0 % by weight, relative to the weight of the sugar. An example of an antimicrobial agent is p-cresol.

In the sugar addition process, sugar is attached to the surface of the first-stage precursor in an amount of 1 % to 30 % by weight, preferably 1 % to 25 % by weight of the raw hide. Adding sugar to the first-stage precursor in this ratio facilitates attachment of the sugar to the surface of the first-stage precursor, is effective in inhibiting the growth of microorganisms, and promotes fermentation in the second fermentation process, thereby providing better curing.

In the second fermentation process, the first-stage precursor to which sugar has been attached as described above is fermented. The fermentation in the second fermentation process may be carried out in a dry or normal humidity space. The second fermentation process may be carried out, for example, in a fixed plant or warehouse, or in a storage unit that also serves as a transport container such as a cargo container for trucks, trains, ships, or airplanes.

In the second fermentation process, fermentation takes place in the raw hide, that is, yeast grows in the raw hide and ethanol is produced by the metabolism of the yeast. According to the present embodiment, the raw hide after sugar has been attached to the surface of the first-stage precursor and fermentation in the second fermentation process has begun (the raw hide after being subjected to the second fermentation process) is referred to as the second-stage precursor. That is, the second-stage precursor is the raw hide containing sugar and the yeast of the genus Saccharomyces, like the first-stage precursor. The raw hide of the second-stage precursor, like that of the first-stage precursor, preferably does not contain salt added for preservation purposes. The second-stage precursor may also include ethanol, depending on the fermentation conditions.

The second-stage precursor in the process of the second fermentation process and the second-stage precursor after the second fermentation process are extremely well cured without the use of salt due to at least one of the effect of reducing free water by the addition of sugar, the effect of yeast growth, or the effect of ethanol produced by fermentation. Therefore, by carrying out the second fermentation process, the effectiveness of the preservation treatment to prevent a change in quality or degradation, such as putrefaction, is further enhanced.

The atmosphere in the room, warehouse, or the like where the second fermentation process is carried out is preferably on the dry side, and specifically, the relative humidity is preferably 30 % to 70 %. The relative humidity of the atmosphere is preferably 40 % to 60 %. The temperature of the space in which the second fermentation process is carried out may be, for example, 20 °C to 40 °C. The temperature of the atmosphere is preferably 20 °C to 30 °C. By carrying out the second fermentation process in such an atmosphere, the effect of the preservation treatment in the second fermentation process is further enhanced.

The period for carrying out the second fermentation process is preferably from 1 day to 50 days, and more preferably from 3 days to 30 days. When the period for carrying out the second fermentation process is one day or longer, preferably three days or longer, the effects of the preservation treatment during and after the second fermentation process can be sufficiently obtained. The period for which the second fermentation process is carried out is 30 days or less, and at most 50 days or less, in order to obtain a sufficiently high effect of the preservation treatment. When the period for carrying out the second fermentation process is from 1 day to 50 days, the effect of the preservation treatment can be maintained for at least 4 weeks to 5 weeks after the second fermentation process. In other words, the second fermentation process makes it possible to preserve the raw hide (the second-stage precursor) for at least about 12 weeks, including the period during which the second fermentation process is being carried out.

In the second fermentation process, the first-stage precursor may be stored by folding so that the sugar-attached surfaces face each other. Specifically, for example, the hides may be folded in half so that the sugar-attached surfaces face each other, and then folded again to form a quarter-fold state. The folded first-stage precursors may be stored in stacks. By folding so that the sugar-attached surfaces face each other, the sugar attached to the first-stage precursor can be prevented from falling off from the surface of the first-stage precursor, and a decrease in the curing effect can be suppressed.

The second-stage precursor is extremely well cured as described above, and therefore the second-stage precursor is suitable for long-term preservation, for example, about 12 weeks, preferably from 1 day to 50 days, long-term transportation between plants located far from each other, and long-term transportation such as import/export from a raw hide producing country to a raw hide using country where the raw hide is processed into leather. As mentioned above, no salt is required in the production of the second-stage precursor. Therefore, wastewater containing a large amount of salt is not generated in the production of the second-stage precursor.

The second fermentation process may be carried out during transportation. In other words, the second fermentation process can also be used as a transportation method to prevent a change in quality or degradation, such as putrefaction, of the raw hide.

In the second fermentation process, when the raw hide has animal hair, an effect of making the animal hair of the second-stage precursor more likely to detach is also achieved. In the second fermentation process, some animal hair detaches as the fermentation progresses. That is, the method for dehairing hide according to the present embodiment may include the second fermentation process. This facilitates the dehairing process (finishing dehairing process) described below.

The dehairing process (finishing dehairing process) is, for example, a process of dehairing the second-stage precursor. The dehairing process may be a process of dehairing the first-stage precursor. In the following, a case where the dehairing process is a process of dehairing the second-stage precursor is described as an example.

In the dehairing process, potassium hydroxide or sodium hydroxide in an amount of 0.3 % to 1.0 % by weight, and sodium sulfide in an amount of 0.8 % to 2.0 % by weight or a mixture of sodium hydrogen carbonate and sodium bicarbonate in an amount of 0.8 % to 2.0 % by weight, each relative to the weight of the raw hide, are added to the second-stage precursor and stirred. In the method for producing leather according to the present embodiment, dehairing is also promoted in the first fermentation process and the second fermentation process, and therefore this dehairing process is a process in which finishing of dehairing is carried out in the method for producing leather according to the present embodiment, or in other words, the finishing dehairing process. The method for dehairing hide according to the present embodiment may include this finishing dehairing process.

The amount of potassium hydroxide or sodium hydroxide added in the dehairing process is preferably 0.6 % to 0.9 %, relative to the weight of the raw hide. Sodium hydroxide is preferably used in the dehairing process.

When sodium sulfide is added in the dehairing process, the amount added is preferably 0.8 % to 1.50 %, relative to the weight of the raw hide.

When a mixture of sodium hydrogen carbonate and sodium bicarbonate is added during the dehairing process, the ratio of sodium hydrogen carbonate to sodium bicarbonate is preferably set to approximately 50:50, and more specifically set to a range from 40:60 to 60:40.

Stirring in the dehairing process may be carried out in a rotating drum, similar to the soaking process. The rotation speed of the drum is 5 revolutions per minute to 12 revolutions per minute, preferably 5 revolutions per minute to 9 revolutions per minute, and more preferably 7 revolutions per minute to 8 revolutions per minute. A stirring time of about 15 minutes is sufficient. The stirring time is preferably 10 minutes to 15 minutes. This dehairing process completely separates the hair from the hide (the second-stage precursor).

In the dehairing process according to the present embodiment, a large amount of water or a large amount of lime (slaked lime, calcium hydroxide) is not used, as in conventional techniques. The dehairing process according to the present embodiment does not require the use of lime, and the process of so-called liming as in conventional techniques is not required. That is, the dehairing process according to the present embodiment does not discharge a large amount of lime sludge as in conventional techniques, and therefore has a low environmental impact. Further, the amount of sodium sulfide used in the dehairing process according to the present embodiment is small.

The desulfurization process is a process of removing sulfur content (sulfur groups) from the first-stage precursor or the second-stage precursor after the dehairing process. In the desulfurization process, an oxidizing agent is added to the first-stage precursor or the second-stage precursor after the dehairing process in an amount of 0.8 % to 2.0 % by weight, relative to the weight of the raw hide, and the mixture is stirred. This removes sodium sulfide and the like. The stirring may be carried out in a rotating drum, similar to the soaking process. The drum rotates at a speed of, for example, 5 revolutions per minute to 12 revolutions per minute.

An example of an oxidizing agent that can be used in the desulfurization process is a peroxide such as H₂S, Na₂O₂, Na₂H₃CO₆, or H₂O₂.

The desulfurization process is carried out for, for example, about 30 minutes to 60 minutes. The desulfurization process normally takes about 45 minutes. The desulfurization process does not need to be time-controlled; it is sufficient to carry out the process until a smell of hydrogen sulfide gas disappears from the first-stage precursor or the second-stage precursor after the dehairing process, or until a color of a liquid seeping out from the first-stage precursor or the second-stage precursor after the dehairing process becomes light brown.

After the desulfurization process, a so-called dealkalization process is carried out in which potassium hydroxide and sodium hydroxide are removed from the first-stage precursor or the second-stage precursor after the dehairing process, using a mixture of weak acids such as acetic acid, citric acid, and formic acid. In this process, a bleaching agent such as sodium hydrogen sulfate may be used in combination, as required. The dealkalization process may be carried out in a drum subsequent to the previous process.

After the dealkalization process, the first-stage precursor or the second-stage precursor can be tanned to be finished into leather (tanned leather). When the raw hide does not have animal hair, the second-stage precursor (the second-stage precursor that has not been subjected to the dehairing process) immediately after the second fermentation process can be tanned to be finished into leather (tanned leather). The tanned leather may be further subjected to dyeing treatment or the like.

As described above, the method for producing leather and the leather precursor are provided that have a low environmental impact and do not require the use of large amounts of salt for preserving raw hide or large amounts of lime or water for dehairing.

### EXAMPLES

### (Example 1)

Raw hides were prepared from cows (but not salted). First, the raw hides were initially washed, weighed and pretreated with soap and soda ash. In the following, when simply referring to the weight of the raw hide, this refers to the weight of the raw hide measured after the initial washing. Thereafter, water (25 °C) having an equal weight to the raw hide and granulated sugar (5 %, 10 %, 15 %, and 20 %, relative to the weight of the raw hide) were placed in containers.

In parallel with the above, a starter was prepared. The starter was prepared by adding 10 g of yeast (Saccharomyces cerevisiae), 5 g of sugar, and 50 ml of warm water (50 °C) to a separate container and allowing fermentation for 20 minutes in a sealed state.

The prepared starter was added to the containers containing the raw hide and the rest, the contents of the containers were stirred, the containers were covered and stored at room temperature, and fermentation of the four samples was initiated. The room temperature was approximately 25 °C to 35 °C, and the relative humidity was 40 % to 70 %. Thereafter, the condition of the raw hides (corresponding to the first-stage precursor) was checked at defined time intervals.

After one day, no detachment of hair was visually observed. Pinching the raw hides or rubbing with the fingertips did not result in hair detachment.

After two days, the hair detachment was the same as on the first day. There was a change in smell compared to the first day. The four samples with different sugar formulations showed similar changes.

After three days, animal hair detachment (hereinafter referred to as dehairing) was observed in thin hair areas such as the abdomen in the samples containing 5 %, 10 %, and 15 % sugar.

After four days, dehairing was observed evenly in thin hair areas for all four samples containing different amounts of sugar.

After five days, all four samples exhibited uniform dehairing in the thin hair areas.

After six days, about 80 % of the hair in each of the four samples was easily removable.

After four weeks, the smell of hydrogen sulfide gas and ammonia began to be detected. Further, a smell began, indicating the breakdown of keratin and globular proteins. The smell of alcohol also increased.

After seven weeks, complete dehairing was observed in all four samples. However, a decrease in tear strength of the hides was also observed.

As described above, the raw hide fermented in the treatment liquid, that is, the first-stage precursor, could be cured and preserved for less than seven weeks without using salt. Further, after fermentation for a defined number of days (for example, three days), the effect of promoting dehairing was observed.

### (Example 2)

Fermentation of four samples was initiated in the same manner as in Example 1, and after 12 hours, the raw hides (corresponding to the first-stage precursor) were squeezed in a press and dewatered. The squeezing ratio was 40 %. The squeezing ratio is the ratio (%) of the weight of the water that had been removed, assuming that the weight of the raw hide containing water immediately before dewatering was 100 %.

After dewatering, the back surface of each raw hide sample was evenly coated with sugar (sucrose) in an amount of 20 % by weight, relative to the weight of the raw hide. Each sample coated with sugar was folded in half with the sugar-coated sides facing each other, then folded again in quarters, stacked, and stored in a dry room (warehouse). The room temperature was approximately 20 °C to 30 °C, and the relative humidity was 40 % to 60 %. Thereafter, the condition of the raw hides (corresponding to the second-stage precursor) was checked at defined time intervals.

After one day, no detachment of hair was visually observed. Pinching the raw hides or rubbing with the fingertips did not result in hair detachment.

After two days, the hair detachment was the same as on the first day. There was a change in smell compared to the first day. The four samples with different sugar formulations showed similar changes.

After three days, animal hair detachment (hereinafter referred to as dehairing) was observed in thin hair areas such as the abdomen in the samples containing 5 %, 10 %, and 15 % sugar.

After four days, dehairing was observed evenly in thin hair areas for all four samples containing different amounts of sugar.

After five days, all four samples exhibited uniform dehairing in the thin hair areas.

After six days, for all four samples, about 80 % of the hair fell out easily, and about 95 % of the hair was in a state where it could be easily removed.

After four weeks, the smell of hydrogen sulfide gas and ammonia began to be detected. Further, a smell began, indicating the breakdown of keratin and globular proteins. The smell of alcohol also increased.

After seven weeks, no deterioration of the leather was visually observed in any of the four samples. No decrease in the tear strength was observed and no deterioration of the hide was visually observed, and therefore it was determined that protein degradation of the raw hide had not progressed.

No difference was observed between the 12 week and 7 week periods.

As described above, even after removal from the treatment liquid, fermentation continued, and the effect of promoting dehairing was obtained. Further, the raw hide after being coated with sugar, that is, the second-stage precursor, could be cured and preserved for at least 12 weeks.

In comparison with the samples of Example 1, the samples of Example 2 exhibited no decrease in the tear strength of the leather after seven weeks.

When raw hide is preserved in the treatment liquid for a long period of time, as in the samples of Example 1, it is thought that fermentation proceeds excessively, producing acids such as acetic acid, causing the treatment liquid to become acidic. It is thought that this is why the tear strength of the samples of Example 1 was reduced due to the acid causing decomposition (hydrolysis) of proteins. However, no such decrease in tear strength of the hides was observed in the samples of Example 2, and therefore it was found that for longer-term preservation of raw hide, it is more preferable to complete the first fermentation process within a defined period, move on to the second fermentation process, and preserve in the second-stage precursor state.

Thus, it was found that, particularly in the state of the second-stage precursor, good preservation is possible at room temperature for at least 12 weeks without deterioration in appearance or physical properties (tear strength) and without the addition of salt.

As described above in Examples 1 and 2, the method for producing leather according to the present embodiment does not require salt to preserve the raw hide, and does not generate waste liquid containing large amounts of salt during the leather production, resulting in a low environmental impact.

It was also found that raw hide preserved as described above (treated in the first fermentation process or the first fermentation process and the second fermentation process) had promoted dehairing during preservation. Therefore, in the dehairing process after the first fermentation process or the second fermentation process, the process of liming as required in a conventional technique is no longer necessary, which reduces the environmental impact. That is, the method for dehairing hides according to the present embodiment does not discharge a large amount of lime sludge, and therefore has a low environmental impact.

When the method for producing leather according to the present embodiment is not used for preservation of raw hide but is used as the method for dehairing according to the present embodiment, the raw hide subjected to the first fermentation process and the second fermentation process may be salted. In such a case, waste liquid containing salt may be generated during the leather production (the process of implementing the method for dehairing according to the present embodiment), but a large amount of lime sludge is not discharged, and the environmental impact is still low.

As described above, the method for producing leather and the leather precursor that have a low environmental impact can be provided.

### (Other embodiments)

(1) According to an embodiment described above, the dehairing process of dehairing the second-stage precursor is described as an example. However, the dehairing process is not limited to dehairing the second-stage precursor. The dehairing process can be carried out as described above for the first-stage precursor. That is, the dehairing process may be, for example, a process of dehairing the first-stage precursor. In such a case, the dehairing process may include a process of adding potassium hydroxide or sodium hydroxide in an amount of 0.3 % to 1.0 % by weight, and sodium sulfide in an amount of 0.8 % to 2.0 % by weight or a mixture of sodium hydrogen carbonate and sodium bicarbonate in an amount of 0.8 % to 2.0 % by weight, each relative to the weight of the raw hide, to the first-stage precursor and stirring the mixture.
(2) According to an embodiment described above, the atmospheric conditions in the first fermentation process and the second fermentation process, and the holding times (fermentation time) required in the first fermentation process are described. However, these described atmospheric conditions and holding times (fermentation time) are not essential requirements. The first fermentation process and the second fermentation process involve yeast growth and metabolism, that is, so-called microbial reactions. Therefore, the requirements regarding the atmospheric conditions and holding time (fermentation time) in the first fermentation process and the second fermentation process only affect the rate at which the microbial reactions progress. In the method for producing leather according to the present embodiment, the effects of the preservation treatment and the dehairing described according to the present embodiment are realized as long as the microbial reactions progress in the first fermentation process and the second fermentation process.

The embodiments disclosed herein are illustrative, and variations as appropriate within the scope of the present disclosure may be made without being limited to the disclosed embodiments.

### INDUSTRIAL APPLICABILITY

The present disclosure is applicable to methods for producing leather and leather precursors.

## Claims

1. A method for producing leather, the method comprising:
a soaking process of immersing a raw hide in a treatment liquid containing a sugar and a yeast of the genus Saccharomyces; and
a first fermentation process of immersing the raw hide in the treatment liquid and fermenting.

2. The method for producing leather according to claim 1, wherein the treatment liquid contains
water in an amount of 50 % to 200 % by weight of the raw hide, and
the sugar in an amount of 1.5 % to 30 % by weight of the raw hide.

3. The method for producing leather according to claim 2, wherein the first fermentation process is carried out in an atmosphere having a temperature of 15 °C to 40 °C and a relative humidity of 30 % to 80 %.

4. The method for producing leather according to claim 3, wherein, in the first fermentation process, the raw hide is kept immersed in the treatment liquid for 2 hours to 72 hours and fermented.

5. The method for producing leather according to any one of claims 1 to 4, the method further comprising:
a dewatering process of dewatering a first-stage precursor obtained by fermenting the raw hide in the first fermentation process;
a sugar addition process of attaching sugar to a surface of the first-stage precursor after the dewatering process; and
a second fermentation process of fermenting the first-stage precursor after the sugar addition process.

6. The method for producing leather according to claim 5, wherein, in the sugar addition process, sugar is attached to the surface of the first-stage precursor in an amount of 1 % to 30 % by weight of the raw hide.

7. The method for producing leather according to claim 6, wherein, in the second fermentation process, the first-stage precursor is fermented
in an atmosphere having a temperature of 20 °C to 40 °C and a relative humidity of 30 % to 70 %,
for a period of 1 day to 50 days.

8. The method for producing leather according to any one of claims 5 to 7, the method further comprising a dehairing process of dehairing a second-stage precursor obtained by fermenting the first-stage precursor in the second fermentation process, wherein,
in the dehairing process,
potassium hydroxide or sodium hydroxide in an amount of 0.3 % to 1.0 % by weight, and
sodium sulfide in an amount of 0.8 % to 2.0 % by weight, relative to the weight of the raw hide,
are added to the second-stage precursor and stirred.

9. The method for producing leather according to claim 8, further comprising a desulfurization process carried out after the dehairing process, wherein,
in the desulfurization process, an oxidizing agent is added to the second-stage precursor in an amount of 0.8 % to 2.0 % by weight, relative to the weight of the raw hide, and stirred.

10. The method for producing leather according to any one of claims 1 to 4, the method further comprising a dehairing process of dehairing the first-stage precursor obtained by fermenting the raw hide in the first fermentation process, wherein,
in the dehairing process,
potassium hydroxide or sodium hydroxide in an amount of 0.3 % to 1.0 % by weight, and
sodium sulfide in an amount of 0.8 % to 2.0 % by weight, relative to the weight of the raw hide,
are added to the first-stage precursor and stirred.

11. The method for producing leather according to claim 10, the method further comprising a desulfurization process carried out after the dehairing process, wherein,
in the desulfurization process, an oxidizing agent is added to the first-stage precursor in an amount of 0.8 % to 2.0 % by weight, relative to the weight of the raw hide, and stirred.

12. The method for producing leather according to any one of claims 1 to 11, the method further comprising preparing a starter comprising the yeast, wherein,
in the process of preparing the starter, 5 g to 10 g of the yeast, 5 g to 10 g of a sugar, and 30 ml to 70 ml of warm water at 40 °C to 60 °C are fermented in a sealed state for 15 minutes to 20 minutes to prepare the starter.

13. A leather precursor comprising a sugar, a yeast of the genus Saccharomyces, and a raw hide.

14. The leather precursor of claim 13, further comprising ethanol.
